

## UNITED STATES PATENT OFFICE

2,350,559

## CRANKCASE INSULATION

Sidney E. Klenitz, New York, N. Y., assignor to  
Pentrathane Products, Inc., Long Island City,  
N. Y., a corporation of New York

No Drawing. Application August 12, 1941,  
Serial No. 406,517.

2 Claims. (Cl. 117—27)

My present invention relates to an insulating material and, more particularly, to an insulating material which is sufficiently flexible and has a sufficiently high K factor and adhesion to enable its use for automotive crankcases and in any other case where a flexible insulation is needed.

While, in the manufacture and construction of motor vehicles of various types, a great deal of emphasis has in the past been placed upon maintaining a definite maximum temperature and preventing the oil or other fluids used in connection with the motor from rising above this maximum temperature, less emphasis has been placed upon the maintenance of a minimum temperature, which will ensure the best operating efficiency of the vehicle.

It is well-known, for instance, that the oil normally used in a vehicle for lubrication will have a consistency or viscosity which will prevent improper filtration by any filtering or cleaning means connected with the vehicle should the oil temperature be too low.

In cold weather, when starting a motor vehicle, the metal parts in the vehicle have all shrunk due to the low temperature. Therefore, all of the gasoline which comes from the carburetor into the motor is not consumed but some of it passes or squirts by the rings and goes down into the crankcase and mixes with the oil, causing dilution, sometimes to the extent of 20 or 25 per cent. Then, in addition, because of this cold condition, water vapor which is always present in the air taken into the motor through the breather of the crankcase goes below the dew point and forms actual water. The water plus the gasoline above-mentioned plus the oil then forms into a soapy mass or sludge. The sludge remains in the crankcase and until the oil attains a temperature of at least 140 degrees F. will not break up. If it is possible to maintain a higher temperature than 140°, then the oil will begin to again pass through the filter and the sludge will break up, the dilution will evaporate and so will part of the water. Sludge is probably the most dangerous condition in automotive problems.

A great amount of radiation of heat in the ordinary motor vehicle is in the crank case itself where the oil collects. In cold weather and particularly during the winter months, the heat in the oil may readily radiate to the outside atmosphere through the metallic crank case, thus leading to the deleterious and adverse effects previously noted.

Various attempts have been made to provide an insulating coating for the surface of the crank

case in order to prevent such radiation. But in every case such insulating coatings have been failures, owing not so much to the fact that they did not insulate properly, but rather because the crank case in a motor vehicle is subject to severe vibration and very great variations in temperature conditions.

This made it almost impossible to economically attach insulation to the crank case itself.

Thus, any insulating coating having a sufficiently high K factor which was applied to the crank case was shaken or dusted off after the motor vehicle had been in use for only a short period of time. Owing to the various stresses in the crank case itself and further owing to the vibration, the insulating material tended to crumble and fall apart.

An object of the present invention is the formation of an insulating coat for surfaces and particularly for surfaces which are in constant vibration, the said insulating coating having a high K factor and nevertheless being flexible and yielding rather than friable or crumbling.

Other attempts to provide an insulation which will have the proper insulating qualities and be sufficiently secure have been so expensive as to be impractical.

I have found that most insulating materials having the requisite insulating properties are rather of a friable or crumbly nature; and hence, if merely caused to adhere by any sizing or glue to a surface, may readily be detached therefrom by constant vibration and severe variations in temperature. This is the primary reason for the failure of prior insulating coatings which have been employed on crank cases of various kinds.

A further object of this invention, therefore, is the combination of an insulating material which may be of a friable or relatively stiff or crumbling character with a matrix of a plastic material which is flexible and resilient in such a manner that the matrix cushions and secures each particle of the insulating material and at the same time causes both the matrix and the insulating material to adhere securely to the surface to be insulated.

A further object of this invention is the provision of a plastic, flexible, insulating coat comprising a quantity of insulating material dispersed in a matrix of flexible plastic adherent material in such a manner that it may yield readily to severe vibrations and severe changes in temperature of the surface to which it is attached, and in such manner that it will remain attached to

such surface under any of the foregoing conditions.

A further object of the present invention is the provision of an insulating coating, for a surface, of such a nature that it will not crumble, rupture or break apart and will adhere to the surface under severe vibratory conditions under severe changes in relative humidity of the adjacent atmosphere and during severe changes in temperature, and so that it will resist weathering.

Still another object of the present invention is the provision of an adherent, resilient, flexible, plastic insulating coating for a surface, said coating consisting of finely divided insulating material, such as vermiculite, embedded in a matrix of rubber, the said rubber matrix positioning and encasing each of the particles of the vermiculite in order to form an insulating mass and also providing an adherent surface for securing to the surface upon which the coating is to be placed.

Another object of the present invention is a method for securing an insulating plastic, resilient, flexible surface or coating to a surface which is to be insulated.

These and many other objects of the present invention will in part be apparent and where not apparent pointed out in the following description:

One example of an embodiment of my invention consists of a plastic coating for a surface wherein the coating consists primarily of powdered vermiculite embedded in a rubber matrix formed from a pre-vulcanized latex such as "Vul-tex." The rubber matrix encases and positions each particle of vermiculite to form a substantially continuous insulating coating, the rubber latex also serving to cause the coating to adhere to the surface to be insulated.

In the actual preparation of the material for application to a surface to be insulated, I first screen the vermiculite to remove the rough particles, particularly where the insulating coating is to be of the order of only  $\frac{1}{8}$ " in thickness.

Should a thicker coating be necessary, then coarser particles may be used. But, in the case of ordinary crank case insulation, I have found that a  $\frac{1}{8}$ " coating over the outer surface is sufficient.

I then prepare a solution of pre-vulcanized latex consisting of 30% solids and 70% water. Ordinarily, the pre-vulcanized latex is securable in commerce as in the form, for instance, of "Vul-tex" which consists of a 60% solution of latex in water.

I dilute this solution so that the proportion of water therein is 70%. I then add a retarder to the liquid latex solution, the said retarder preferably consisting of a casein which is added in an amount of the order of 1% by volume to the solution. The retarder may be procurable as an ordinary article of commerce in the form for instance of "Casco" cement.

The retarder is not absolutely essential to the formation of the plastic coating but I have found that while the plastic coating hereinafter described will ordinarily set in 15 minutes and thus presents problems in its application, the addition of the retarder delays the setting time by one hour and thus allows sufficient time for the coating to be applied.

Hence, while the retarder is not essential to the insulating coating which is eventually to be formed, it is, in ordinary practice, quite necessary to use the retarder in order to permit the working and formation of the insulation.

I then combine the vermiculite and the solution above noted as follows: To one-half gallon of the pre-vulcanized latex casein solution I add 22 ounces of powdered vermiculite. The powder is stirred slowly into the liquid and is thoroughly combined therewith. The mixture is then ready for application and the application thereof should be completed within one hour after the mixture has been formed.

It is essential that the powder be stirred or poured into the liquid. If the reverse operation were performed, simply a ball of rubber would be obtained, since the rubber would then start to oxidize in the air and would dehydrate.

All of the foregoing operations are performed at normal atmospheric temperatures.

In actual commercial use, I prepare the liquid solution of pre-vulcanized latex or "Vul-tex" and casein in the proper proportions and package these in half-gallon cans. I also prepare 22-ounce packages of powdered vermiculite. The materials for the insulating coating are thus prepared and packaged in separate form.

The consumer, when he is ready to apply the coating, stirs the powdered vermiculite into the liquid solution and spreads the material on the surface to be insulated with a knife or a spatula or with his hands.

Normally, I have found that a  $\frac{1}{8}$ " thick coating provides sufficient insulation for an automobile crankcase.

The coating sets within one hour to a condition where it is a relatively solid mass and achieves a sufficiently complete set in four hours to permit its use. In twelve hours the final set is achieved and the insulating coating has reached its fullest K factor.

The insulating coating, when it has set, consists of powdered insulating material such as vermiculite embedded in a rubber matrix formed by the pre-vulcanized latex solution.

The embedding of the powdered vermiculite in the rubber matrix ensures that all of the insulating material will always be adherent to the surface and the rubber matrix itself is adherent to the surface, thus causing the entire mass to adhere.

Owing to the embedding of the insulating material in the flexible rubber matrix, the insulating coating is resilient and flexible and will yield readily to any vibrational forces rather than crumble by reason thereof.

The preparation of this type of coating in this manner and the embedding of the insulating material in the rubber matrix by the method herein set forth permits the utilization of any type of insulating material in powdered form no matter how friable or crumbly the same may be.

Thus, the disadvantages of prior insulating coatings for crank cases are obviated since the material cannot crumble nor can particles thereof be torn away by vibration.

In the actual preparation and securing of the insulating coating to a crank case, I have found that the best results are achieved by placing a thin film of cement or glue on the crank case surface before the coating is applied in the manner above set forth.

The coating is thereafter applied and adheres to the surface not merely by reason of adhesion of the latex but also by reason of the cement. This adherence has been tested and has been found to resist a force of 1000 pounds per square foot.

After the coating is applied and has set, I have found that best results and protection from mud and weathering may be obtained by shellacking the surface, and, specifically, I have obtained the best results by use of two coats of an orange shellac. 5

The K factor of the insulating coating may be improved by the addition of more insulating particles or materials. However, the proportions above set forth have been found by experiment 10 to be the best.

The more vermiculite there is in the coating, the greater the insulating powers and the more latex found in the coating, the greater the adhesive powers. Hence a compromise must be effected between the two and sufficient latex is used to ensure the adherence of all of the particles of vermiculite to the coating so that the same will not powder or dust off. 15

I have found that the K factor of the insulating coating formed on a crank case in the manner above described is higher than that of any other plastic insulation which is used for severe vibration. 20

It will not crumble, rupture, or break apart 25 and can, if desired, be removed in warm weather, though I have found that best results are obtained by leaving the insulation on the crankcase permanently.

In the actual application of my insulating coating to a crankcase, I have found that it is best to apply the coating to a warm crankcase and the best results are obtained by leaving it in a warm atmosphere with good air circulation. 30

Additional coatings of my insulating material 35 may be applied on top of prior coatings.

In some forms, I have found that a mixture of powdered vermiculite and powdered concrete produces the best results. It should be remembered that many other types of powdered or 40 fibrous insulating materials may be utilized in the coating and dispersed within the rubber matrix in the manner above described.

In the winter time, in the use of automobiles on start-stop vehicles, oil will rarely warm up to the optimum operating temperature. Oil will not function properly in a motor vehicle unless it reaches a temperature of 140° F. 45

Many instances have occurred in which not even an oil temperature of 90° F. has been 50 reached in the winter.

Various tests with crankcases protected by my insulating surface have shown that the heat imparted to the oil by the engine and by the circulating water is retained so efficiently in the crankcase (when my insulating coating is used) that the minimum safe operating temperature of 140° F. for the oil is very quickly reached and very efficiently maintained. 55

In addition to utilizing other forms of insulating material as insulating particles to be dispersed in the matrix, various other types of ad-

herent, flexible, yielding materials may be used to form the matrix and I am not necessarily limited to pre-vulcanized latex. Other types of latex may be used and other plastics of a yielding resilient adhering material may be used. 60

Primarily my invention is intended for use in the insulation of crankcases for automotive vehicles, since in such uses the most severe vibrations occur and hence make necessary a plastic, resilient, yielding, flexible, adherent coating which will not crumble or easily be removed. However my insulating coating may obviously be as readily used in connection with other types of insulating problems and may, for instance, be used as pipe insulation, wall insulation, container insulation or for other insulation purposes. 15

While I have herein set forth the proportions which I have found useful for obtaining optimum results both with respect to insulating properties and flexibility and adherence, it must be remembered that these results are obtained by a compromise of all of the elements of the coating. 20

Greater insulating properties might be obtained if the avoidance of crumbling were not an important problem or if adherence and flexibility and resilience were not important. And of course greater adherence, resilience and flexibility might be obtained where insulation is not important. 25

Thus, the quantities may be varied in accordance with the particular use desired. 30

For purposes of use in connection with crank case insulation the foregoing proportions have however been found to be the best compromise to produce results which are commercially acceptable. 35

In describing my invention, I have necessarily set forth but a few illustrations of the basic principles involved.

Many other elements of my invention should now be obvious to those skilled in the art and many variations and modifications thereof should also be clear. 40

Accordingly, I prefer to be bound not by the specific disclosures herein but only by the appended claims. 45

I claim:

1. The method of forming an adherent, resilient, flexible insulating coating for the surface of a crankcase, comprising the steps of stirring 22 ounces of powdered vermiculite into one-half gallon of a 30% suspension of pre-vulcanized latex, spreading the mass thus formed upon the surface and permitting the mass to dry. 50

2. The method of forming an adherent, resilient, flexible insulating coating for the surface of a crankcase, comprising the steps of stirring 22 ounces of powdered vermiculite into one-half gallon of a 30% suspension of pre-vulcanized latex containing 1% by volume of casein, spreading the mass thus formed upon the surface and permitting the mass to dry. 55

SIDNEY E. KIENITZ.